

## UNITED STATES PATENT OFFICE

2,170,024

## CELLULOSE ESTERS AND METHOD

Winfield W. Heckert, Arden, Del., assignor to E. I.  
du Pont de Nemours & Company, Wilmington,  
Del., a corporation of Delaware

No Drawing. Application April 15, 1937,  
Serial No. 137,147

9 Claims. (Cl. 8—26)

This invention relates to cellulosic filaments, threads, films and fabrics which have increased elasticity and/or crease-resistance and to processes for preparing such filaments, threads, films and fabrics.

This invention has as an object the preparation of crease-resistant cellulosic filaments, threads, films and fabrics. A further object is the preparation of cellulosic filaments, threads, films and fabrics which have increased elasticity. A still further object is the preparation of crease-resistant cellulosic filaments, threads, films and fabrics which have a substantial degree of elasticity. A still further object is the manufacture of threads which will give knitted fabrics with greater elasticity. Another object is to improve the elasticity of fabrics knitted from viscose rayon. Another object is to render cellulosic threads and fabrics insoluble in solvents. Other objects will appear hereinafter.

These objects are accomplished by subjecting a cellulosic filament, thread, film or fabric to the action of a bifunctional reagent taken from the class consisting of carboxylic acid esterification agents and etherification agents. In a more limited sense they are accomplished by reacting a bifunctional reagent taken from the class consisting of carboxylic acid esterification agents and etherification agents until substantial proportions of both functional groups of the bifunctional reagent added have reacted and the product has attained increased crease-resistant and elastic properties.

In the present application bifunctional reagents are defined as those reagents which react bifunctionally with cellulose. It is known that certain compounds which are bifunctional in form do not react bifunctionally with cellulose except when combined with other reaction inducing, but not catalytic means, these means being called in the cellulose are "impellers". Thus, phthalic anhydride ordinarily reacts with cellulose as a monofunctional reagent to give a derivative which is soluble in dilute alkalis, i. e. one in which one carboxyl of the phthalic anhydride is combined with the cellulose, the second carboxyl remaining free. If, in addition to the phthalic anhydride, an impeller (e. g., benzoyl chloride) is present in the proportion of two or more mols benzoyl chloride to one mol phthalic acid, a dianhydride is formed which is capable of reacting bifunctionally with cellulose to form an insoluble derivative.

The amount of bifunctional reagent to be used in the reaction mixture may be varied quite

widely and depends upon a number of factors, including the result desired, the nature of the cellulosic starting material, and the bifunctional reagent used. In practice, as will be seen from the examples which follow, I treat the cellulosic fabric, etc., with a limited amount of the bifunctional reagent (e. g., dianhydride of a dicarboxylic acid) and then limit the amount of the reagent substituted in the cellulose nucleus by stopping the reaction when the desired increase in elasticity has been attained.

From the above it will be seen that, because of the number of variables involved, it is not possible to set forth all possible combinations of conditions for success. For the operator skilled in the art it will be sufficient to explain that the cellulosic fiber, fabric, etc., is treated with a small amount of a bifunctional esterification or etherification reagent under conditions known to the art to be suitable for the purpose, and that the reaction is terminated when the required increase in elasticity has been attained.

The invention will be further illustrated but is not intended to be limited by the following examples in which the quantities are stated in parts by weight.

## Example I

A solution of sebacic-benzoic anhydride is prepared by dissolving 16.2 parts of sebacic acid in 98 parts of pyridine and adding 11.2 parts of benzoyl chloride. The pyridine hydrochloride which precipitates is filtered off and the solution diluted to 125 parts with pyridine. The cellulosic thread, film or fabric, such as skeins of viscose rayon, regenerated cellulose films or viscose rayon hose, are activated by soaking in water, centrifuging and replacing the water with pyridine. They are then heated with 12 to 18 parts of the above solution at a temperature of about 70° C. for two to three days at which time the fiber or fabric will have been found to have combined with approximately  $\frac{1}{4}$  equivalent of sebacic acid per glucose residue. The reaction time may be increased if a higher degree of substitution is desired. Continual agitation of the reaction mixture is desirable in order to secure uniform esterification. Thus, skeins may be arranged on screen trays in a tank and the reaction mixture circulated over them by removing the fluid at the bottom and pumping it back into the tank at the top. At the completion of the reaction time the skeins, films or hose are washed with alcohol and then scoured with soap in the usual manner. Hose are boarded over hosiery forms.

Such treatment will have been found to im-

part crease-resistance to the yarn. Samples reacted to varying degrees of combined sebacic acid had the following angles of crease:

| 5  | Equivalents of sebacic acid/glucose residue | Angle of crease | Degrees |     |
|----|---------------------------------------------|-----------------|---------|-----|
|    |                                             |                 | 95      | 107 |
| 10 | Control.....                                | 95              | 95      | 95  |
|    | 0.10.....                                   | 107             | 107     | 107 |
|    | 0.24.....                                   | 109             | 109     | 109 |
|    | 0.46.....                                   | 117             | 117     | 117 |
|    | 0.64.....                                   | 120             | 120     | 120 |

The "angle of crease" was measured by winding the thread over a double-edged blade while supporting a 50-gram weight, holding for thirty minutes, releasing the weight, unwinding the "angles", cutting these apart, allowing them to recover for ten minutes, and then measuring the recovered angle with a protractor. Perfect crease-resistance by this method would have been indicated by an angle of crease of 180°. If the time of creasing were increased, all of the "angles of crease" would have been smaller, or if the time had been shortened they would have been larger.

If these yarns are knitted into fabrics, the fabrics are found to have improved elasticity, i. e., they recover more completely after stretching than do similar fabrics knitted from untreated yarn. Thus, a fabric knitted from viscose rayon esterified with 0.46 equivalent of sebacic acid had an elastic recovery of 63% when stretched 50% for three minutes at 74% relative humidity. The corresponding viscose rayon fabric had an elastic recovery of 42%. Those treated in the above manner show similar improvements in elastic recovery from stretch.

It will be noted that the esterifying power of benzoic acid for cellulose is very low, so that in the above treatment cellulose sebacate is produced almost exclusively. Two mols of benzoyl chloride are used with each mol of sebacic acid so that both carboxyl groups of the sebacic acid combine with the cellulose.

#### 45 Example II

Thirty-one and two-tenths (31.2) parts of succinic acid (0.264 mol) were dissolved in 1100 parts of pyridine. Seventy-four and three-tenths (74.3) parts of benzoyl chloride (0.528 mol) were added slowly, with stirring. The mixture was cooled for several hours, filtered and diluted to 1200 parts with pyridine. In case any water is present it is necessary to use an excess of benzoyl chloride to react with it.

A skein of 450 meters of 150 denier gel viscose rayon (rayon which had never been dried) was dehydrated with pyridine and then placed in a jar with 200 parts of the above reaction mixture. The jar was placed in an oven at 70° C. on a swinging tray which caused the reaction liquid to be constantly agitated. After eighteen hours the skein was removed and washed thoroughly with warm water and dried. The increase in weight indicated at 0.99 equivalent of succinic acid per glucose residue had combined with the cellulose. Its angle of crease was 122° compared with 99° for an untreated control. It was an entirely different product from that obtained by reacting a similar skein with succinic anhydride. The latter product was very sensitive to moisture, had an extremely poor wet strength and was soluble in dilute alkali. The former was not soluble in dilute alkali and was less water-sensitive than the untreated yarn.

#### Example III

A stock solution of benzoic adipic anhydride was prepared by dissolving 73 parts of adipic acid in 686 parts of pyridine. One hundred forty and five-tenths (140.5) parts of benzoic chloride were added, with stirring. After cooling for several hours, the solution was filtered.

A skein of 450 meters of 150 denier gel viscose rayon was dehydrated with pyridine and reacted with a mixture of 62 parts of the above solution diluted with 38 parts of pyridine. The reaction was carried out under conditions similar to that described in Example II. The product was found to have combined with 0.31 equivalent of adipic acid per glucose residue. The angle of crease of this sample was 110° compared with 95° for the control.

#### Example IV

A skein of cotton thread was reacted with 1 mol of phthalic anhydride and 1 mol of benzoyl chloride in pyridine for sixty-four hours at 50° C. The sample after washing and drying had an angle of crease of 153° (creased fifteen minutes) compared with 134° for the untreated yarn.

#### Example V

A cellulose acetate thread containing 1.38 mols of combined acetic acid per C<sub>6</sub> unit of cellulose was prepared by esterifying 450 meters of 150 denier gel rayon with 200 parts of 25% acetic anhydride in pyridine for about five hours at 70° C. A solution of sebacic-benzoic anhydride was prepared by dissolving 101 parts of sebacic acid in 1100 parts of pyridine, adding 140.5 parts of benzoyl chloride with stirring, cooling, filtering and diluting to 1150 parts with pyridine. The cellulose acetate skein was reacted with 150 parts of this solution for forty hours at 70° C. The skein was washed with alcohol and water, and dried. Its increase in weight indicated that 0.33 equivalent of sebacic acid had combined with the cellulose. The yarn now had an angle of crease of 141° (creased fifteen minutes) compared with 120° for the corresponding viscose yarn and was insoluble in all solvents which did not destroy the ester linkages.

#### Example VI

One hundred (100) parts of cotton filter cloth are steeped in 50% caustic and then pressed to 500 parts. This is treated with 228 parts of dichlorodimethyl ether in 400 parts of benzene in an autoclave for six hours at 150° C. The product still retains its form and is insoluble in all organic solvents and even cuprammonium solution, and may therefore be used for filtering such solutions.

Various types of cellulosic filaments, threads, films and fabrics may be used as starting materials in accordance with my invention. Thus cellulose acetate, propionate, butyrate, etc., and mixed lower carboxylic acid esters, methyl cellulose, ethyl cellulose, etc., and mixed ethers, cellulose glycolic acid, regenerated cellulose such as viscose rayon and cotton when in the form of filaments, threads, films and fabrics may be treated to produce products having increased crease-resistance and elasticity and insolubility. In the preferred embodiment of the invention, the threads, fabrics, etc., are treated in accordance with the invention and the end-point of the reaction is carefully controlled to give any desired degree of increased elasticity. The process has particular utility in the treatment of viscose rayon skeins or fabrics with bifunctional esterify-

ing agents, and this embodiment represents the most important feature of the invention.

The suitable bifunctional reagents include any etherifying agent or any esterifying agent which 5 reacts bifunctionally toward cellulose and preferably such reagents containing two or more carbon atoms. I find that the most effective type of bifunctional etherifying agent has the functional groups attached to primary carbon atoms. Polyfunctional etherification agents containing more 10 than two functional groups may also be used, but for most purposes are less satisfactory than bifunctional reagents. Among the etherifying agents which may be used are ethylene dichloride, 15 dichlorodiethyl ether, xylylene dibromide, trimethylene chloride, omega-omegadichlorodipropyl ether, and beta-beta'-dichlorodiethyl sulfide.

Polyfunctional esterifying agents which may be 20 used to advantage include dianhydrides or dichlorides derived from dibasic acids or the equivalent thereto, i. e., dibasic acids with an impeller, the latter being in amount greater than molar in relation to the dibasic acid. Among the dibasic 25 acids which may be used in combination with an impeller are succinic, adipic, sebacic, phthalic and octadecamethylene dicarboxylic acid. It will be noted that the agents of this invention result in products having primary valence bonds between the nuclei of cellulose and the agent.

This invention is useful in a number of ways, for instance, in the production of crease-resistant 30 textiles, for improving the elasticity of fabrics such as rayon hose, and for rendering threads and fabrics inert to solvents. The threads and fabrics are new and have innumerable commercial uses.

Crease-resistant and fabric elasticity are very 35 important properties of textile materials composed of cellulose derivatives. This invention has the advantage that fabrics having the just-mentioned properties may be easily and economically obtained. An additional advantage lies in the fact that knitted fabrics which are crease-resistant and have good elastic properties may be 40 easily obtained.

The above examples and description are intended to be illustrative only. Any modification

of or variation therefrom which conforms to the spirit of the invention is intended to be included within the scope of the claims.

I claim:

1. The process of increasing the elasticity of 5 cellulose material which comprises reacting a cellulose filament, thread, fabric or film with a bifunctional esterification agent of the group consisting of dianhydrides and dichlorides of dicarboxylic acids, and terminating the reaction 10 when the desired degree of increase in elasticity is obtained.

2. The process of increasing the elasticity of 15 cellulose material which comprises reacting a cellulose filament, thread, film or fabric with a dianhydride of a dibasic carboxylic acid and terminating the reaction when the desired degree of elasticity is attained.

3. The process for enhancing the crease-resistance 20 of viscose materials which comprises reacting a viscose rayon filament, thread or fabric with a dianhydride of a dibasic carboxylic acid until a substantial increase in crease-resistance is obtained.

4. The process according to claim 1 wherein 25 the dianhydride results from the reaction of a dicarboxylic acid and benzoyl chloride.

5. The process according to claim 2 wherein the 30 dianhydride results from the reaction of phthalic acid and benzoyl chloride.

6. The process according to claim 2 wherein the 35 dianhydride results from the reaction of adipic acid and benzoyl chloride.

7. The process according to claim 2 wherein the dianhydride results from the reaction of sebacic acid and benzoyl chloride.

8. Cellulose filaments, threads, films and fabrics reacted with a dianhydride of a dibasic carboxylic acid, said products being characterized by substantially increased elasticity and crease-resist- 40 ance.

9. Regenerated cellulose filaments, threads and fabrics reacted with a dianhydride of a dibasic carboxylic acid, said products being characterized by substantially increased elasticity and 45 crease-resistance.

WINFIELD W. HECKERT.

CERTIFICATE OF CORRECTION.

Patent No. 2,170,024.

August 22, 1939.

WINFIELD W. HECKERT.

It is hereby certified that error appears in the printed specification of the above numbered patent requiring correction as follows: Page 1, first column, line 41, for the word "impellers" read impellors; page 2, first column, line 65, for "at" read that; and second column, line 5, for "benzoil" read benzoyl; line 31, for "dernier" read denier; page 3, first column, lines 22 and 26, for "impeller" read impellor; line 38, for "Crease-resistant" read Crease-resistance; and second column, line 9, claim 1, for "dianhydrides" read dianhydrides; line 25, claim 4, for the claim reference numeral "1" read 2; and that the said Letters Patent should be read with this correction therein that the same may conform to the record of the case in the Patent Office.

Signed and sealed this 26th day of September, A. D. 1939.

(Seal)

Henry Van Arsdale,  
Acting Commissioner of Patents.